

Nov. 9, 1926.

1,606,282

C. A. WITTER

PROCESS OF MAKING PIPE FLANGES

Filed Oct. 29, 1924



Fig. 1.

Fig. 2.



Fig. 3.



Fig. 4.



Fig. 5.

INVENTOR  
C. A. WITTER

WITNESS  
Gustav Henglinger

BY  
Synnestvedt & Lechner  
ATTORNEYS

## UNITED STATES PATENT OFFICE.

CLAUDE A. WITTER, OF PHILADELPHIA, PENNSYLVANIA.

## PROCESS OF MAKING PIPE FLANGES.

Application filed October 29, 1924. Serial No. 746,455.

This invention relates to the process of forging a plurality of pipe flanges of commercial size from a single ingot.

In general my invention contemplates the speeding up of production and the elimination of a large percentage of the waste incident to processes now being employed.

I aim to eliminate such waste by forging a plurality of pipe flanges from a single ingot whereby the amount of material allowed for draft is reduced, that is to say no allowance for draft is needed on the outermost diameters of the pipe flanges, with the exception of the largest flange.

It is apparent that a great saving of time is afforded by my process in that a plurality of flanges may be produced in practically the same time as one flange is produced by existing methods which are known to me.

How these and various other objects and advantages can be realized through my invention will appear from my description hereinafter of the best process for the purpose known to me.

In the drawings Fig. 1 is a perspective view of the ingot;

Figs. 2, 3, and 4 show results obtained by successive forging steps; and,

Fig. 5 shows a plurality of finished pipe flanges made from a single ingot.

The ingot 7 may be in the form of a cylinder or prism and is of a volume equal to that of the flanges which it is desired to produce, plus certain allowances for draft and finish.

This ingot 7 is forged to the approximate contour which the plurality of flanges would take, if placed one inside of the other as shown in Fig. 4, the dotted lines representing the finished pipe flanges. The forging may be accomplished by using any standard form of forging press preferably of the steam hammer type.

In the drawings I have shown three steps of forging to bring the ingot to the above mentioned state, the first step being one of flattening the ingot and increasing its diameter, the second step being one of further forging the flattened ingot to a configuration roughly resembling a plurality of concentric pipe flanges and of increasing its diameter, and the third step being one of forging it to a shape more nearly approximating a plurality of finished concentric pipe flanges.

During forging the humps 8 shown in Fig. 3 become the upstanding parts 10 of the flanges and the portions 9 become flattened forming the bases 11 of the flanges.

As is well known in this art it is necessary to allow sufficient draft so that the forging may be easily separated from the die, which allowances I have shown on the outer diameter 12 and on the faces 13 and 14 of the upstanding parts 10 of the flanges.

I have found that a plurality of various sized flanges can be produced one inside the other, in such a way that by removing the amount of metal required for draft on the surfaces 14, the outer flange will have the proper inside diameter and the adjacent inner one will have the proper outside diameter. Removal of this metal may be accomplished either by shearing or by a parting tool. In cases where a more finished product is desired I propose to machine the outer surfaces 12 and the upper and lower surfaces 15 and 16 respectively. The hole 17 in the innermost flange may be machined or sheared.

It is to be understood that all of the flanges may be separated in one operation or by successive operations as desired.

When forging pipe flanges, one at a time, it is necessary to make allowance for draft both at its innermost and outermost diameters, while by my process, allowance at the outermost diameters of the various flanges making up a set is eliminated with the exception of course of the largest pipe flange.

The surfaces 13 and 18 are forged to actual dimension and need no machining, unless a "finish all over" is particularly specified.

I claim:

1. The process of making pipe flanges which consists in forging an ingot to the approximate contour of a plurality of substantially concentric connected pipe flanges, in forging some of the surfaces to size, and in separating said flanges so as to finish the inside diameters and the outside edges thereof.

2. The process of making a plurality of pipe flanges of successively increasing diameters from a single ingot, which consists in forging the ingot to a flat shape of approximately the diameter of the largest flange, of then forging it to the approximate contour

of a plurality of substantially concentric pipe flanges connected by the draft allowance and in then separating said pipe flanges by removing the draft allowance.

5. The process of making pipe flanges which consists in forging an ingot to a shape having a flat bottom and an upper face hav-

ing a plurality of concentric upstanding ribs and in separating said ribs at a point adjacent the inside diameters thereof.

10 In testimony whereof, I have hereunto signed my name.

C. A. WITTER.